

## UNITED STATES PATENT OFFICE

2,257,437

## CAST METAL ARTICLES

Hanley H. Weiser, Prince Bay, Staten Island, N. Y., assignor to Nassau Smelting & Refining Company, Incorporated, New York, N. Y., a corporation of New York

No Drawing. Application October 31, 1939,  
Serial No. 302,119

3 Claims. (Cl. 75—154)

This invention relates to cast metal articles, and more particularly to articles cast from copper-tin-silicon alloys which are highly resistant to corrosion and also have unusually high elongations before rupture under high tensile stresses.

Increasing efforts are being made, especially in industry based on chemical engineering procedures, to ensure safety in all possible ways. Apparatus employed in chemical industries particularly make extensive use of pipes and fittings, such as valves, which not only are normally subjected to high pressure and the corrosive action of fluids passing through them, but which also may be subject to sudden and incalculable internal pressures of greater magnitude due to accidental stoppages, unintended chemical reactions, or other causes. Consequently a search has been made for materials for making such members, which shall not only have high tensile strength and resistance to corrosion, but which shall also yield slowly and deform extensively before ultimate rupture under excessive tensile stresses, thus frequently perhaps relieving the stresses before rupture actually occurs.

An object of the present invention is to provide cast articles having the properties of high tensile strength, high resistance to corrosion and unusually great elongation before rupture when subjected to occasional high tensile stresses.

With the above and other objects in view, the invention may be embodied in an article cast of an alloy consisting essentially of

|              |              |
|--------------|--------------|
| Per cent     |              |
| Silicon..... | 2.00 to 3.75 |
| Tin.....     | 0.25 to 1.50 |

and the balance copper except for insignificant amounts of other substances having no harmful effects.

Other objects and features of the invention will appear from the following detailed description of embodiments thereof.

Many alloys, generally called silicon bronzes, have been known for a long time and variously described. Usually they are essentially binary copper-silicon alloys or ternary copper-silicon alloys in which the third characteristic metal is tin or zinc or iron or manganese, although a wide variety of alloys having these and other metals as constituents are known. These alloys frequently are satisfactorily corrosion resistant for many uses in chemical industry but they lack some or all of the desirable characteristics exhibited by the alloys of the present invention

which render them especially suitable for making cast articles which may be subjected to sudden and large stresses.

Characteristics that are desirable in alloys for use in making cast products of this nature are fluidity when molten in order to cast well and especially to reproduce effectively fine detail in the mold, low wetting power when molten in order that molding sand may not adhere to the solidified casting as it does with many bronze and brass alloys, the peculiar mixture of toughness and severability which renders the material machinable when solid, high tensile strength, and, above all, a high degree of elongation before rupture under excessive tensile stresses.

It has been discovered that articles cast from an alloy of essentially the following basic composition possess the desired characteristics in an unusually high degree:

|              |      | Minimum | Optimum | Maximum |
|--------------|------|---------|---------|---------|
|              |      | Percent | Percent | Percent |
| Silicon..... | 2.00 | 3.25    | 3.75    |         |
| Tin.....     | 0.25 | 1.00    | 1.50    |         |

and the balance copper except for insignificant amounts of other substances having no harmful effects.

Iron or manganese or both may be present in amount up to a total of 0.50% without materially affecting the desirable properties either favorably or unfavorably. Cadmium and nickel are somewhat detrimental and should be held under 0.10% if present at all. Aluminum is detrimental in any amount and should therefore not be present.

The alloys described are remarkably fluid when molten and make clean, sharp castings free from adherent sand. They possess high tensile strength and they are highly corrosion resistant, showing a possession of this characteristic, under test, to a somewhat higher degree than comparable alloys to be found generally available commercially.

It is, however, in elongation before rupture under tensile stress that these alloys are particularly notable. Comparable commercial silicon bronzes show elongations generally of the order of 10% to 40%, with occasional specimens having elongations as high as 50% or a little over, the tests being made on sand cast specimens and the elongations being measured over an original two inch length. But the particular alloys here in question show elongations of which

the following results, obtained in experimental tests, are typical:

| Melt No. | Percent Si | Percent Sn | Tensile strength in pounds per square inch | Percent elongation in 2 inches |
|----------|------------|------------|--------------------------------------------|--------------------------------|
| 1.       | 2.49       | 1.05       | 50,510                                     | 69.0                           |
| 2.       | 2.73       | 1.05       | 50,780                                     | 72.1                           |
| 3.       | 3.55       | 0.35       | 52,210                                     | 76.5                           |
| 4.       | 3.37       | 0.78       | 54,645                                     | 68.0                           |

In each case the balance of the alloy consisted of copper except for harmless impurities. Each of the above figures for tensile strength and elongation is the average of tests on five separate specimens sand cast from the same melt, and tested without any heat treatment or other modification of the cast structure.

Apparently there is within a closely circumscribed and limited range of values of the silicon and tin in the series of ternary copper-silicon-tin alloys, the small group of alloys containing from about 2.00% to about 3.75% of silicon, from about 0.25% to about 1.50% of tin, and the balance, except for negligible impurities, copper, which group exhibits elongations having values from two to four times as great as other alloys of similar composition. As noted above, these elongations are shown by the alloys as cast in sand, without any special subsequent treatment such as annealing or other heat treatment to develop this character, and as measured over an original length of two inches. Hence, articles cast from the alloys will have these elongations without further treatment.

Cast articles embodying the invention will be of particular value when used under conditions where sudden shocks of considerable magnitude may be expected. Thus, for example, they are especially suited for the manufacture of pipes and fittings for apparatus to be used in chemical industry and which, by accident, may be subjected to excessive internal pressures. In such cases, if these articles are cast from the alloys of the invention, they will yield slowly and extensively before finally rupturing and so may well prevent or at least minimize damage to their surroundings even if their own usefulness be destroyed. It will be, of course, necessary that such articles show a high degree of resistance to corrosion; and have high tensile strength and these particular alloys have these characteristics as well as the unusual high elongation and toughness.

So far the alloys of the invention have been considered as applied to the direct casting of articles to be used without extensive further treatment. The alloys, however, are adaptable for use also where an article requiring considerable machining after casting is to be produced. While the alloys as described are machinable, they are somewhat difficult to machine satisfactorily. It has been found that their machinability may be improved by adding a small amount of lead thereto. When modified by the addition of not over about 0.5% and preferably about 0.25% of lead, they retain their toughness, strength and remarkable elongation, and in addition are freely machinable.

Thus an alloy whose composition was

|         | Per cent |
|---------|----------|
| Silicon | 3.20     |
| Tin     | 1.12     |
| Lead    | 0.24     |

and the balance copper except for insignificant amounts of other harmless substances, showed, as the average of five specimens, a tensile strength of 51,310 pounds per square inch and an elongation of 62.4%, and was satisfactorily machinable.

Alloys of copper with silicon and tin are old and well known in the art and have been used extensively in the manufacture of wrought products. However, it is believed that until the present discovery, the wholly unexpected and extremely useful properties of the specific alloys disclosed herein were entirely unknown. Furthermore, the peculiar value of cast articles and parts capable of being subjected to sudden tensile stress without rupture was also not known. In accordance with the invention, such articles are simply, cheaply and reliably made by direct casting from these alloys without need for further apparatus or procedures for subsequent treatment. Since the invention is believed to reside only in cast articles made from the specific alloys and having the extraordinary properties described, no claim is made to the alloys as such.

It is, of course, to be understood that by cast articles, as this term is used herein and in the annexed claims, is meant articles having predetermined configurations which are designed to be utilized in the form in which they are cast for purposes where the peculiar and hitherto unknown properties of these alloys are especially desirable. It is not intended that the claims shall be interpreted to cover ingots, billets, bars, slabs or other shapes into which metals produced in bulk are formed for the purpose of providing masses which may be conveniently stored and handled and which are designed to be subjected to further treatments or operations, such as rolling, forging, extrusion, drawing, etc., in which their shapes will be entirely altered.

What is claimed is:

1. Corrosion resistant, cast metal articles designed to be used as cast without further fabrication except machining, having elongations of upwards of 55% before rupture under tensile stress, and made of an alloy consisting of silicon 2.00% to 3.75%, tin 0.25% to 1.50%, and the balance substantially all copper.

2. Corrosion resistant, cast metal articles designed to be used as cast without further fabrication except machining, having elongations of upwards of 60% before rupture under tensile stress, and made of an alloy consisting of silicon about 3.25%, tin about 1.00%, and the balance substantially all copper.

3. Corrosion resistant, cast metal articles designed to be used as cast without further fabrication except machining, having elongations of upwards of 75% before rupture under tensile stress, and made of an alloy consisting of silicon about 3.50%, tin about 0.35%, and the balance substantially all copper.